

May 6, 1930.

R. A. GORTNER ET AL

1,757,768

PURIFIED FIBER

Original Filed Sept. 2, 1925



INVENTORS

Ross Aiken Gortner and  
Walter Fred Hoffman.

BY

Penrice Davis Marvin & Edwards

ATTORNEYS

## UNITED STATES PATENT OFFICE

ROSS AIKEN GORTNER AND WALTER FRED HOFFMAN, OF ST. PAUL, MINNESOTA, ASSIGNEES TO THE NORTHWEST PAPER COMPANY, OF CLOQUET, MINNESOTA, A CORPORATION OF MINNESOTA

## PURIFIED FIBER

Original application filed September 2, 1925, Serial No. 54,003. Divided and this application filed January 30, 1926. Serial No. 84,863.

This invention relates to a method for purifying vegetable fibers, and specifically wood fibers and paper pulp. The paper pulp may be cooked or given other chemical treatments, 5 such as bleaching, before being treated by our process. The wood fibers may be shredded or in the form of chips. The object of this invention is to remove, by means of the electric current, a large portion of the ash 10 present in vegetable fibers and also to remove organic coloring matter and impurities usually present in these materials. In addition to the object above disclosed, our invention further improves and purifies such fibers so 15 that they remain white and do not turn yellow when subjected to the action of the atmosphere at elevated temperatures. A further object is to make a purified paper pulp which retains its original strength in comparison 20 with the weakened pulps purified by drastic chemical treatments.

Our method is an improvement over the old methods of treating pulp and vegetable fibers with alkalies and acids of various kinds 25 to remove organic and inorganic impurities contained therein. Our simplified method has the advantage in that the individual fibers are not subjected to the drastic action of the chemicals used for purifying heretofore used, 30 and therefore results in a much higher yield and quality of product, not only from the standpoint of color, but also from the standpoint of physical properties. Our process can be carried out in a simple type of electrolytic cell.

In the accompanying drawing there is illustrated, in diagrammatic form, a simple electrolytic cell which we preferably use to carry out our present invention. In the drawing, 1 is a suitable container, which may be constructed of wood and made water proof and tight in the usual manner. A typical cell which has been used successfully for carrying out our invention but which may be modified 40 in its dimensions and construction to suit conditions, has the following interior dimensions: 10" long, 6" wide, and 5" deep. Partitions 4 and 5 are membranes which are permeable to the colloids which are present in vegetable fibers, but which will retain the

fibers. We have found that ordinary 10 ounce canvas is suitable for wood pulp but we are not limited to this material. Any material which has the property of retaining the fibers to be purified but which allows the impurities to pass through and which is not readily destroyed by the contents or the action of the cell, is suitable. If it is desirable to remove electrolytes and retain the colloids such as organic coloring matter and colloidal 55 silica, a diaphragm impermeable to colloids is used.

The diaphragms 4 and 5 are mounted across the cell so as to divide the cell into three compartments, 6, 7 and 8; 7 being the anode and 8 the cathode compartment, the direction of flow of the electric current being shown by the arrows. The compartments may be of equal capacity or the central compartment 60 may be of much greater or smaller capacity 55 than either of the anode and cathode compartments. In the anode and cathode compartments suitable electrodes 2 and 3 are placed. The anode is preferably made of a graphite plate and in the specific cell described is about 4½" x 6" in area. Due to the presence of chlorides and sulphates, graphite is most suitable, due to the disintegrating action on other materials. The cathode 65 70 75 80 85 90 95 3 may be of graphite or may be of metals such as iron, copper, etc., which are not attacked.

It is not necessary to have the diaphragms placed as is shown in the illustration. Any arrangement which will allow the liquid about the electrodes to be readily renewed may be used. In the operation of the cell the vegetable fibers, such as paper pulp, are introduced into the central compartment 6 in the form of a slurry which may contain about 5 to 10 per cent of pulp. If wood chips are used the central compartment is filled with them. The chips may be wet or dry. The cell is then filled with water to a suitable height to prevent overflowing. Heating the contents of the cell results in a more rapid purification than is obtained at room temperature, due to the greater mobility of the ions and colloids at the higher temperatures.

A suitable temperature is one which approaches the boiling point of water.

The electrodes are attached to any suitable source of direct current, and in the cell illustrated, which is about 10" long, a pressure of about 220 volts has been used to carry out the desired reaction for ordinary wood pulp. This high pressure is desirable since the electrolyte consists of water, the conducting ions being supplied by the impurities in the water, the ash in the fibers, and the salts remaining in the pulp after the washing operations in the pulp mill. Chemicals may be added to the water. All electrolytes are decomposed and are removed from the anode and cathode compartments. The current, when chemicals are not added, has been less than one ampere for the cell illustrated, or less than 5 amperes per sq. ft. of the cross sectional area of the pulp in a plane parallel to the electrodes. The higher the ash content, the greater the conductivity, thereby increasing the current density. The current gradually drops and the liquid in one or both electrode compartments, assumes a dark color. The liquid in the anode compartment contains the anions such as Cl and  $\text{SO}_4$  and negatively charged colloids, while the cathode compartment liquid contains positively charged colloids and the cathions such as calcium, sodium, and iron. The coloring matter in the water of the electrode compartments is probably due to the lignins and other organic compounds such as are contained in black liquor (not completely washed out after the cooking operation in the digestors).

The impure liquids accumulated at the electrodes in the anode and cathode compartments are preferably changed from time to time to prevent diffusion back into the pulp or vegetable fibers contained in the central compartment. Although the impure liquids may be changed intermittently a continuous stream of fresh water, which may be hot, can be run into these compartments, as through pipes 9 and 10, and the impure water removed by suitable overflow openings 11 and 12. Not only may the impure water be removed continuously, but the pulp may also be added to and removed from the central compartment to make the operation continuous.

The pulp is subjected to the electric current until it has reached the desired purity, or if a highly purified pulp is desired, the electrolysis is continued until the resistance of the cell becomes so high that the current drops to almost zero, our measurements indicating below .10 ampere per square foot of cross sectional area of the pulp. This low conductivity indicates a high degree of purity.

The finished pulp may be given a final washing with pure water.

The pulp which is subjected to the electric current is whitened or bleached considerably,

if it has not been previously bleached, and very appreciable amounts of coloring materials may be removed from pulps that have been chemically bleached. The whitening is no doubt due to the removal of the lignin or other organic compounds. Bleaching may precede or follow the electrolytic treatment. In addition the ash content of the fiber or pulp has been decreased so that it may be below .05 per cent and in some cases we have found it to be as low as .031 per cent. The original ash in this pulp was 1.43 per cent. The electric current removes a large part of the inorganic impurities, especially those of the alkaline earths, alkalies, and heavy metals such as iron, but does not fully remove the silica. We have found that the ash which is retained consists essentially of silica with some traces of iron. Highly refined pulps such as are used in the quantitative filter papers differ from our product in that the ash consists of complex alkaline earth compounds and contains little silica.

Ordinary bleached sulphite pulp of a good white color, when subjected to a temperature of 60 to 70 degrees C. for 100 hours turns yellow. This same pulp when subjected to our treatment yields a dark liquor at the anode and the color is improved. The pulp stays pure white when heated at 60 to 70 degrees C. for 100 hours. The pulp purified by our method thus has a special application to products which must not color when subjected to heat, which also indicates that they will not turn yellow with age.

Our method may also be used to whiten unbleached fibers which may have been cooked and washed to remove most of the chemicals and impurities.

Authorities are generally of the opinion that the non-cellulosic materials or impurities occurring in vegetable fibers including wood, are adsorbed by the cellulose. Such adsorbed impurities should be capable of being removed when subjected to the action of the electric current in water solution. This theory is borne out by our results. Most of the inorganic impurities are ionized and under the influence of the electric current travel to the oppositely charged poles at either end of the cell, resulting in the presence of chlorine and sulphate ions at the anode and the basic sodium, calcium and iron ions at the cathode. Colloidal silica particles of such size that they show cataphoresis are removed by our process. Our experiments show that silica is not entirely removed though it possibly may be removed under certain conditions. Such colored organic compounds as are colloidal will possess either a positive or a negative charge, the sign of the charge depending upon the hydrogen ion concentration of the liquid in the central compartments, and under the influence of the electrical current will travel either to the cath-

ode or the anode, as evidenced by the water becoming dark colored in the cathode or anode compartment as the electrolysis proceeds. The cellulose is normally negatively charged and tends to travel to the anode, but is stopped by the canvas or other diaphragm and piles up against this diaphragm. If the cellulose becomes dense enough, water may even pile up in the cathode chamber. Some 10 experiments show that it is possible to give the cellulose a positive charge so that it will travel toward the cathode chamber. In general our process removes electrolytes, and such colloids as may migrate by cataphoresis and which will pass through the membrane used. A membrane impermeable to colloids will only remove electrolytes from the fiber or pulp, and thus reduces the ash content by electro-dialysis.

20 While the hemi-cellulose and the degraded celluloses (oxy-cellulose and hydro-cellulose) are considered to be adsorbed by the cellulose these apparently are not removed, or only partially removed, by the electrolytic action.

25 It is our belief that these cellulose compounds and modifications are so intimately connected with the pure cellulose as to approach chemical combination so that they cannot be removed, or are only partially removed, under 30 the conditions outlined. By electrolyzing the pulp in a water suspension to which chemicals, such as acids or alkalis have been added, the results indicate that cellulose-like impurities are removed. Tests have shown 35 that when a bleached pulp containing oxy-cellulose is subjected to our process, the oxy-cellulose is still present after this treatment, though the coloring compounds have been removed and the ash has decreased to less than .05 per cent.

40 While we have described a specific form of apparatus for carrying out our process, we do not wish to be limited to this form but claim broadly the process of removing electrolytes and organic and inorganic impurities, part or all of which may have been adsorbed on the cellulose fibers, by passing an electric current through vegetable fibers in water suspension and removing such impurities as are accumulated at or near the electrodes. The diaphragms are used to keep the impurities away from again contaminating the pulp. Since the pulp usually has a 45 tendency to migrate toward the anode, it may be possible to dispense with the diaphragm at the cathode, under certain conditions, and if the cellulose is positively charged, it may not be necessary to have a diaphragm at the anode. Our invention applies to vegetable 50 fibers in general, and specifically to wood fibers, whether in aggregates as in wood chips or disintegrated in the form of pulp, and wood pulp and paper pulp containing 55 vegetable fibers of various kinds, cooked or uncooked, and bleached or unbleached. This

application is a division of our co-pending application, Serial No. 54,003, filed September 2, 1925.

We claim:

1. A purified wood fiber substantially free from adsorbed inorganic impurities except silica. 70
2. Cellulose substantially free from adsorbed inorganic impurities except silica.
3. Paper pulp derived from wood substantially free from inorganic impurities except silica. 75
4. Paper pulp substantially free from impurities except hemi-cellulose, degraded cellulose and adsorbed mineral matter not exceeding .05 percent and consisting essentially of silica. 80
5. Vegetable fiber substantially free from impurities except hemi-cellulose, degraded cellulose and adsorbed mineral matter consisting essentially of silica. 85
6. Cellulose derived from wood substantially free from impurities except hemi-cellulose, degraded cellulose and adsorbed mineral matter not exceeding .05 percent and consisting essentially of silica. 90
7. A paper pulp containing less than .05 percent of ash, said ash consisting essentially of silica. 95
8. A paper pulp which does not color on heating at 60 to 70 degrees C. for 100 hours, said pulp containing hemi-cellulose, degraded cellulose, and less than .05 percent of ash consisting essentially of silica. 100
9. A paper pulp consisting essentially of wood fibers, substantially free from impurities except hemi-cellulose, degraded cellulose and silica. 105
10. A paper pulp consisting essentially of wood fibers, substantially free from impurities except hemi-cellulose, degraded cellulose, and adsorbed mineral matter, said mineral matter not exceeding .05 percent and consisting essentially of silica. 110
11. A vegetable fiber consisting essentially of wood fibers, containing hemi-cellulose and degraded cellulose, but substantially free from adsorbed inorganic impurities, electrolytes, and other colloidal organic impurities. 115
12. Vegetable fiber consisting essentially of wood fibers, containing an ash consisting essentially of silica. 120
13. A paper pulp consisting essentially of wood fibers, containing less than .05 percent of ash, said ash consisting essentially of silica. 125
14. Vegetable fiber consisting essentially of wood fibers which does not color on heating at 60 or 70 degrees C. for 100 hours, said fiber containing hemi-cellulose, degraded cellulose, and less than .05 percent of ash consisting essentially of silica. 130
15. A paper pulp which does not color on heating at 60-70° C. for 100 hours, said pulp 135

containing less than .05% of ash, consisting essentially of silica.

16. Vegetable fiber consisting essentially of wood fiber, which does not color on heating at 60-70° C. for 100 hours, said fiber containing less than .05% ash consisting essentially of silica.

In testimony whereof we affix our signatures.

**10 ROSS AIKEN GORTNER.**  
**WALTER FRED HOFFMAN.**

**15****20****25****30****35****40****45****50****55****60****65**